

[54] MONOFUNCTIONAL AMINES AS  
ADJUVANT FOR LIQUID ELECTROSTATIC  
DEVELOPERS[75] Inventors: Lyla M. El-Sayed; James R. Larson,  
both of West Chester, Pa.; Torence J.  
Trout, Yorklyn, Del.[73] Assignee: E. I. du Pont de Nemours and  
Company, Wilmington, Del.

[21] Appl. No.: 178,962

[22] Filed: Apr. 7, 1988

[51] Int. Cl.<sup>5</sup> ..... G03G 9/12[52] U.S. Cl. ..... 430/115; 430/904;  
524/901

[58] Field of Search ..... 430/115, 114, 904

## [56] References Cited

## U.S. PATENT DOCUMENTS

|           |         |                 |       |           |
|-----------|---------|-----------------|-------|-----------|
| 3,417,019 | 12/1968 | Beyer           | ..... | 252/62.1  |
| 3,427,258 | 2/1969  | Trease          | ..... | 430/107 X |
| 3,565,805 | 2/1971  | Jones et al.    | ..... | 430/108   |
| 3,770,638 | 11/1973 | Chechak         | ..... | 430/106   |
| 3,844,966 | 10/1974 | Nelson          | ..... | 430/114   |
| 3,900,413 | 8/1975  | Metcalfe et al. | ..... | 430/115   |
| 4,014,856 | 3/1977  | Gilliams et al. | ..... | 252/62.1  |

|           |         |                  |       |          |
|-----------|---------|------------------|-------|----------|
| 4,024,292 | 5/1977  | Lu et al.        | ..... | 427/17   |
| 4,058,470 | 11/1977 | Moschovis et al. | ..... | 252/62.1 |
| 4,097,391 | 6/1978  | Moschovis et al. | ..... | 252/62.1 |

Primary Examiner—J. David Welsh

[57]

## ABSTRACT

Electrostatic liquid developer having improved negative charging characteristics consisting essentially of

- (A) nonpolar liquid having a Kauri-butanol value of less than 30, present in a major amount,
- (B) thermoplastic resin particles having an average by area particle size of less than 10  $\mu\text{m}$ ,
- (C) charge director compound, and
- (D) at least one soluble solid or liquid organic monofunctional amine compound of the formula:  $\text{R}_n\text{NH}_{3-n}$  wherein R is alkyl, cycloalkyl or alkylene, or substituted alkyl, the alkyl, cycloalkyl, alkylene or substituted alkyl group being of 1 to 50 carbon atoms, and n is an integer of 1 to 3.

Optionally, a colorant, e.g., a pigment; metallic soap, adjuvant can be present. The electrostatic liquid developer is useful in copying, making proofs including digital color proofs, lithographic printing plates, and resists.

18 Claims, No Drawings

# MONOFUNCTIONAL AMINES AS ADJUVANT FOR LIQUID ELECTROSTATIC DEVELOPERS

## TECHNICAL FIELD

This invention relates to an electrostatic liquid developer having improved charging characteristics. More particularly this invention relates to an electrostatic liquid developer containing as a constituent a mono-functional amine compound.

## BACKGROUND ART

It is known that a latent electrostatic image can be developed with toner particles dispersed in an insulating nonpolar liquid. Such dispersed materials are known as liquid toners or liquid developers. A latent electrostatic image may be produced by providing a photoconductive layer with a uniform electrostatic charge and subsequently discharging the electrostatic charge by exposing it to a modulated beam of radiant energy. Other methods are known for forming latent electrostatic images. For example, one method is providing a carrier with a dielectric surface and transferring a preformed electrostatic charge to the surface. Useful liquid toners comprise a thermoplastic resin and dispersant nonpolar liquid. Generally a suitable colorant is present such as a dye or pigment. The colored toner particles are dispersed in the nonpolar liquid which generally has a high-volume resistivity in excess of  $10^9$  ohm centimeters, a low dielectric constant below 3.0 and a high vapor pressure. The toner particles are less than  $10 \mu\text{m}$  average by area size. After the latent electrostatic image has been formed, the image is developed by the colored toner particles dispersed in said dispersant nonpolar liquid and the image may subsequently be transferred to a carrier sheet.

Since the formation of proper images depends on the differences of the charge between the liquid developer and the latent electrostatic image to be developed, it has been found desirable to add a charge director compound to the liquid toner comprising the thermoplastic resin dispersant nonpolar liquid and generally a colorant. Such liquid toners, while developing good quality images, still do not provide the quality images or extended machine run stability required for certain end uses e.g., optimum machine performance in digital color proofing, office copying, etc. As a result much research effort has been expended in providing new type charge directors and/or charging adjutants for electrostatic liquid toners. Higher quality image development of latent electrostatic images is still desired.

It has been found that the above disadvantages can be overcome and improved electrostatic liquid developers prepared which have improved image quality on latent electrostatic images.

## DISCLOSURE OF THE INVENTION

In accordance with this invention there is provided an electrostatic liquid developer having improved negative charging characteristics consisting essentially of

(A) a nonpolar liquid having a Kauri-butanol value of less than 30, present in a major amount,

(B) thermoplastic resin particles having an average by area particle size of less than  $10 \mu\text{m}$ ,

(C) a charge director compound, and

(D) at least one organic monofunctional amine compound of the formula:  $R_n\text{NH}_{3-n}$  wherein R is alkyl, cycloalkyl, alkylene, or substituted alkyl, said alkyl,

cycloalkyl, alkylene or substituted alkyl group being of 1 to 50 carbon atoms, and n is an integer of 1 to 3.

Throughout the specification the below-listed terms have the following meanings:

In the claims appended hereto "consisting essentially of" means the composition of the electrostatic liquid developer does not exclude unspecified components which do not prevent the advantages of the developer from being realized. For example, in addition to the primary components, there can be present additional components such as colorants, e.g., pigments: metallic soaps, adjuvants, fine particle size oxides, etc.

Charge director (c) may be referred to as a nonpolar liquid soluble ionic compound.

Conductivity is the conductivity of the developer measured in picomhos (pmho)/cm at 5 hertz and 5 volts.

The electrostatic liquid developer, as defined above, comprises four primary components more specifically described below. Additional components, in addition to the four primary components, include but are not limited to: colorants such as pigments or dyes, which are preferably present, metallic soaps, adjuvants, fine particle size oxides, metals, etc.

The dispersant nonpolar liquids (A) are, preferably, branched-chain aliphatic hydrocarbons and more particularly, Isopar®-G, Isopar®-H, Isopar®-K, Isopar®-L, Isopar®-M and Isopar®-V. These hydrocarbon liquids are narrow cuts of isoparaffinic hydrocarbon fractions with extremely high levels of purity. For example, the boiling range of Isopar®-G is between 157° C. and 176° C. Isopar®-H between 176° C. and 191° C. Isopar®-K between 177° C. and 197° C., Isopar®-L between 188° C. and 206° C., Isopar®-M between 207° C. and 254° C. and Isopar®-V between 254.4° C. and 329.4° C. Isopar®-L has a mid-boiling point of approximately 194° C. Isopar®-M has a flash point of 80° C. and an auto-ignition temperature of 338° C. Stringent manufacturing specifications, such as sulfur, acids, carboxyl, and chlorides are limited to a few parts per million. They are substantially odorless, possessing only a very mild paraffinic odor. They have excellent odor stability and are all manufactured by the Exxon Corporation. High-purity normal paraffinic liquids, Norpar®12, Norpar®13 and Norpar®15, Exxon Corporation, may be used. These hydrocarbon liquids have the following flash points and auto-ignition temperatures:

| Liquid     | Flash Point (°C.) | Auto-Ignition Temp (°C.) |
|------------|-------------------|--------------------------|
| Norpar® 12 | 69                | 204                      |
| Norpar® 13 | 93                | 210                      |
| Norpar® 15 | 118               | 210                      |

All of the dispersant nonpolar liquids have an electrical volume resistivity in excess of  $10^9$  ohm centimeters and a dielectric constant below 3.0. The vapor pressures at 25° C. are less than 10 Torr. Isopar®-G has a flash point, determined by the tag closed cup method, of 40° C. Isopar®-H has a flash point of 53° C. determined by ASTM D 56. Isopar®-L and Isopar®-M have flash points of 61° C., and 80° C., respectively, determined by the same method. While these are the preferred dispersant nonpolar liquids, the essential characteristics of all suitable dispersant nonpolar liquids are the electrical volume resistivity and the dielectric constant. In addition,

tion, a feature of the dispersant nonpolar liquids is a low Kauri-butanol value less than 30, preferably in the vicinity of 27 or 28, determined by ASTM D 1133. The ratio of thermoplastic resin to dispersant nonpolar liquid is such that the combination of ingredients becomes fluid at the working temperature.

Useful thermoplastic resins or polymers include: ethylene vinyl acetate (EVA) copolymers (Elvax® resins, E. I. du Pont de Nemours and Company, Wilmington, Del.), copolymers of ethylene and an  $\alpha,\beta$ -ethylenically unsaturated acid selected from the group consisting of acrylic acid and methacrylic acid copolymers of ethylene (80 to 99.9%)/acrylic or methacrylic acid (20 to 0%)/alkyl (C<sub>1</sub> to C<sub>5</sub>) ester of methacrylic or acrylic acid (0 to 20%), polyethylene, polystyrene, isotactic polypropylene (crystalline), ethylene ethyl acrylate series sold under the trademark Bakelite® DPD 6169, DPDA 6182 Natural and DTDA 9169 Natural by Union Carbide Corp., Stamford, CN; ethylene vinyl acetate resins, e.g., DQDA 6479 Natural and DQDA 6832 Natural 7 also sold by Union Carbide Corp.; Surlyn® ionomer resin by E. I. du Pont de Nemours and Company, Wilmington, DE. etc. Preferred copolymers are the copolymer of ethylene and an  $\alpha,\beta$ -ethylenically unsaturated acid of either acrylic acid or methacrylic acid. The synthesis of copolymers of this type are described in Rees U.S. Pat. No. 3,264,272, the disclosure of which is incorporated herein by reference. For the purposes of preparing the preferred copolymers, the reaction of the acid containing copolymer with the ionizable metal compound, as described in the Rees Patent, is omitted. The ethylene constituent is present in about 80 to 99.9% by weight of the copolymer and the acid component in about 20 to 0.1% by weight of the copolymer. The acid numbers of the copolymers range from 1 to 120, preferably 54 to 90. Acid No. is milligrams potassium hydroxide required to neutralize 1 gram of polymer. The melt index (g/10 min) of 10 to 500 is determined by ASTM D 1238 procedure A. Particularly preferred copolymers of this type have an acid number of 66 and 60 and a melt index of 100 and 500 determined at 190° C., respectively.

In addition, the resins have the following preferred characteristics:

1. Be able to disperse any colorant, e.g., pigment, metallic soap, adjuvant, etc., that may be present,
2. Be substantially insoluble in the dispersant liquid at temperatures below 40° C., so that the resin will not dissolve or solvate in storage,
3. Be able to solvate at temperatures above 50° C.,
4. Be able to be ground to form particles between 0.1  $\mu\text{m}$  and 5  $\mu\text{m}$ , in diameter,
5. Be able to form a particle (average by area) of less than 10  $\mu\text{m}$ . e.g., determined by Horiba CAPA-500 centrifugal automatic particle analyzer, manufactured by Horiba Instruments, Inc., Irvine, Calif.: solvent viscosity of 1.24 cps solvent density of 0.76 g/cc, sample density of 1.32 using a centrifugal rotation of 1,000 rpm, a particle size range of 0.01 to less than 10  $\mu\text{m}$ , and particle size cut of 1.0  $\mu\text{m}$ ; and about 30  $\mu\text{m}$  average particle size, e.g., determined by Malvern 3600 E particle sizer as described below.
6. Be able to fuse at temperatures in excess of 70° C.

By solvation in 3, above, the resins forming the toner particles will become softened swollen or gelatinous.

As indicated above, another instrument for measuring average average particle sizes is a Malvern 3600E Particle Sizer manufactured by Malvern. Southborough,

Mass. which uses laser diffraction light scattering of stirred samples to determine average particle sizes. Since this instrument and the Horiba CAPA-500 described above use different techniques to measure average particle size the readings differ. The following correlation of the average size of toner particles in micrometers ( $\mu\text{m}$ ) for the two instruments is:

|    | Value Determined By<br>Malvern 3600 E Particle Sizer | Expected Range For<br>Horiba CAPA-500 |
|----|------------------------------------------------------|---------------------------------------|
| 10 | 30                                                   | 9.9 ± 3.4                             |
|    | 20                                                   | 6.4 ± 1.9                             |
| 15 | 15                                                   | 4.6 ± 1.3                             |
| 15 | 10                                                   | 2.8 ± 0.8                             |
|    | 5                                                    | 1.0 ± 0.5                             |
|    | 3                                                    | 0.2 ± 0.6                             |

This correlation is obtained by statistical analysis of average particle sizes for 67 liquid electrostatic developer samples (not of this invention) obtained on both instruments. The expected range of Horiba values was determined using a linear regression at a confidence level of 95%. In the specification and appended claims the particle size values are as measured using the Horiba instrument unless otherwise indicated.

Suitable charge director compounds (C), which are used in an amount of 0.1 to 1000 mg/g, preferably 1 to 500 mg/g developer solids, include: lecithin, neutral Calcium Petronate®, neutral Barium Petronate®, neutral Barium Petronate®, oil-soluble petroleum sulfonate, manufactured by Sonneborn Division of Witco Chemical Corp., New York, N.Y., glyceride types disclosed in Chan et al., U.S. Ser. No. 125, 503 filed Nov. 25 1987, the disclosure of which is incorporated herein by reference, e.g., sodium salts of phosphated mono- and diglycerides with unsaturated and saturated acid substituents. A preferred type of glyceride charge director is the alkali metal salt. e.g., Na, of a phosphoglyceride, e.g., Emphos® D70-30C. Witco Chemical Corp., New York, N.Y., which is a sodium salt of phosphated mono- and diglycerides.

The fourth component of the electrostatic liquid developer is at least one organic monofunctional amine compound (D), of the formula: R<sub>n</sub>NH<sub>3-n</sub> wherein R is alkyl, cycloalkyl, or alkylene, or substituted alkyl. e.g., halogen such as Cl, Br, F, I; aryl, e.g., benzyl; said alkyl, cycloalkyl, alkylene, or substituted alkyl group being of 1 to 50 carbon atoms, and n is an integer of 1 to 3. The amine compound which can be a liquid at ambient temperature, or is soluble in the nonpolar liquid, is preferably thoroughly dispersed throughout the developer. The sole active substituent present on the amine is the amine group. Examples of monofunctional amines include: hexylamine, laurylamine, dibutylamine, tributylamine, 2-aminoheptane, 4-aminoheptane, 2-amino-3,3-dimethylbutane, amylamine, 2-aminopentane, cyclooctylamine cyclopentylamine, dicyclohexylamine, diethylcyclohexylamine, dihexylamine, diisobutylamine, cyclohexylamine, 2-ethylhexylamine, 1-hexadecylamine, isoamylamine, 1-methylbutylamine, N-methylcyclohexylamine, 3-methylcyclohexylamine, 1-methylheptylamine, N-methyldibutylamine, N-methyloctadecylamine, octadecylamine, tert-octylamine, tridecylamine undecylamine, trisoamylamine, trihexylamine, trioctylamine, N,N-diisopropylethylamine 3-aminoheptane, N,N-dimethylhexylamine, diocylamine, dipentylamine, dipropylamine, dodecylamine, N-ethyl-dicyclohexylamine, 1-ethylpropylamine N-methyl-

butylamine, 2-methylbutylamine, 2-methylcyclohexylamine, 4-methylcyclohexylamine N-methylcyclodecylamine, N-methyldiethylamine, nonylamine, octylamine, 1-tetradecylamine, tridodecylamine, triamylamine, triethylamine triisooctylamine, tripentylamine, 4-t-butylcyclohexylamine 6-chloro-1-hexylamine, 4-chloro-1-hexylamine, 5-fluoro-1-pentylamine, 6-bromo-1-hexylamine, 6-phenyl-1-hexylamine, benzylamine, 4-methylbenzylamine, 3-amino-propene, 4-amino-1-butene 5-amino-1-pentene, etc. The monofunctional amine is used in an amount of 0.1 to 1000 mg/g, preferably 1 to 500 mg/g developer solids.

Components (A) and (B) are present in the electrostatic liquid developer in the following amounts.

Component (A): 99.9 to 85% by weight, preferably 99.5 to 98% by weight; and

Component (B): 0.1 to 15% by weight, preferably 0.5 to 2% by weight. The amounts of components (C) and (D) in the developer are set out above and are not included in considering weight of developer solids.

As indicated above, additional components that can be present in the electrostatic liquid developer are colorants, such as pigments or dyes and combinations thereof, which are preferably present to render the latent image visible, though this need not be done in some applications. The colorant e.g., a pigment, may be present in the amount of up to about 60 percent by weight or more based on the weight of the resin. The amount of colorant may vary depending on the use of the developer. Examples of pigments are: Monastral® Blue G (C.I. Pigment Blue 15 C.I. No. 74160), Toluidine Red Y (C.I. Pigment Red 3), Quindo® Magenta (Pigment Red 122), Indo® Brilliant Scarlet (Pigment Red 123 C.I. No. 71145), Toluidine Red B (C.I. Pigment Red 3), Watchung® Red B (C.I. Pigment Red 48), Permanent Rubine F6B13-1731 (Pigment Red 184), Hansa® Yellow (Pigment Yellow 98), Dalamar® Yellow (Pigment Yellow 74, C.I. No. 11741), Toluidine Yellow G (C.I. Pigment Yellow 1), Monastral® Blue B (C.I. Pigment Blue 15), Monastral® Green B (C.I. Pigment Green 7), Pigment Scarlet (C.I. Pigment Red 60), Auric Brown (C.I. Pigment Brown 6), Monastral® Green G (Pigment Green 7), Carbon Black, Cabot Mogul L (black Pigment C.I. No. 77266) and Sterling NS N 774 (Pigment Black 7, C.I. No. 77266).

Fine particle size oxides, e.g., silica, alumina, titania, etc.; preferably in the order of 0.5  $\mu\text{m}$  or less can be dispersed into the liquefied resin. These oxides can be used alone or in combination with the colorants. Metal particles can also be added.

Metallic soap, e.g., aluminum tristearate, aluminum distearate, barium, calcium lead and zinc stearates; cobalt, manganese, lead and zinc linoleates; aluminum, calcium and cobalt octoates, calcium and cobalt oleates zinc palmitate, calcium, cobalt, manganese, lead and zinc naphthenates, calcium, cobalt, manganese, lead and zinc resinate, etc., can be dispersed into the liquefied resin. The metallic soap is dispersed in the resin as described in Trout U.S. Pat. No. 4,707,429.

There can be present in the liquid electrostatic developers various adjuvants, e.g., as described in Mitchell U.S. Pat. No. 4,631,244 and 4,663,264, Taggi U.S. Pat. No. 4,670,370, Larson and Trout U.S. Pat. No. 4,681,831, Larson U.S. Pat. No. 4,702,985, and Assignee's U.S. Patent Application Ser. No. 854,610 filed Apr. 22, 1986 now U.S. Pat. No. 4,734,352, the disclosures of which are incorporated herein by reference.

The pigment when present in the thermoplastic resin is present in an amount of 1% to 60% by weight preferably 1 to 30% by weight. The metallic soap, when present, is useful in an amount of 0.01 to 60 percent by weight based on the total weight of the developer solids.

The particles in the electrostatic liquid developer have an average by area particle size of less than 10  $\mu\text{m}$ , preferably the average by area particle size is less than 5  $\mu\text{m}$ . The resin particles of the developer may or may not be formed having a plurality of fibers integrally extending therefrom although the formation of fibers extending from the toner particles is preferred. The term "fibers" as used herein means pigmented toner particles formed with fibers, tendrils, tentacles, threadlets, fibrils, ligaments hairs, bristles, or the like.

The electrostatic liquid developer can be prepared by a variety of processes. For example, into a suitable mixing or blending vessel, e.g., attritor, heated ball mill, 20 heated vibratory mill such as a Sweco Mill manufactured by Sweco Co., Los Angeles, CA, equipped with particulate media for dispersing and grinding, Ross double planetary mixer manufactured by Charles Ross and Son, Hauppauge, N.Y. etc. are placed the above- 25 described ingredients. Generally the resin, dispersant nonpolar liquid and optional colorant are placed in the vessel prior to starting the dispersing step although after homogenizing the resin and the dispersant nonpolar liquid the colorant can be added. The dispersing step is 30 generally accomplished at elevated temperature, i.e., the temperature of ingredients in the vessel being sufficient to plasticize and liquefy the resin but being below that at which the dispersant nonpolar liquid degrades and the resin and/or colorant decomposes. A preferred 35 temperature range is 80 to 120° C. Other temperatures outside this range may be suitable, however, depending on the particular ingredients used. The presence of the irregularly moving particulate media in the vessel is preferred to prepare the dispersion of toner particles. 40 Other stirring means can be used as well, however, to prepare dispersed toner particles of proper size, configuration and morphology. Useful particulate media are particulate materials, e.g., spherical, cylindrical, etc. taken from the class consisting of stainless steel, alumina, ceramic, zirconium, silica, and sillimanite. Carbon 45 steel particulate media is useful when colorants other than black are used. A typical diameter range for the particulate media is in the range of 0.04 to 0.5 inch (1.0 to  $\sim 13$  mm).

After dispersing the ingredients in the vessel until the desired dispersion is achieved typically 1 to 2 hours with the mixture being fluid, the dispersion is cooled, e.g., in the range of 0° C. to 50° C. Cooling may be accomplished, for example, in the same vessel, such as 55 the attritor, while simultaneously grinding in the presence of additional nonpolar liquid with particulate media to prevent the formation of a gel or solid mass; without stirring to form a gel or solid mass, followed by shredding the gel or solid mass and grinding, e.g., by 60 means of particulate media in the presence of additional nonpolar liquid; or with stirring to form a viscous mixture and grinding by means of particulate media in the presence of additional nonpolar liquid. Cooling is accomplished by means known to those skilled in the art and is not limited to cooling by circulating cold water or a cooling material through an external cooling jacket adjacent the dispersing apparatus or permitting the dispersion to cool to ambient temperature. The resin 65

solidifies or precipitates out of the dispersant during the cooling. Toner particles of average particle size (by area) of less than 10  $\mu\text{m}$ , are formed by grinding for a relatively short period of time.

After cooling and separating the dispersion of toner particles from the particulate media, if present, by means known to those skilled in the art, it is possible to reduce the concentration of the toner particles in the dispersion. The concentration of the toner particles in the dispersion is reduced by the addition of additional dispersant nonpolar liquid as described previously above. The dilution is normally conducted to reduce the concentration of toner particles to between 0.1 to 3 percent by weight, preferably 0.5 to 2 weight percent with respect to the dispersant nonpolar liquid. One or more charge director compound, of the type set out above, can be added to impart a negative charge. The addition may occur at any time during the process. If a diluting dispersant nonpolar liquid is also added, the charge director compound can be added prior to, concurrently with or subsequent thereto. The monofunctional compound is preferably added subsequent to the developer being charged. For example, with certain acid-containing resins the monofunctional amine compound when present during the hot dispersing step could give undesirable crosslinking of the resin.

#### INDUSTRIAL APPLICABILITY

The electrostatic liquid developers of this invention demonstrate improved charging qualities such as improved stabilized conductivity over liquid toners containing standard charge directors or other known additives. The developers of this invention are useful in copying e.g., making office copies of black and white as well as various colors; or color proofing, e.g., a reproduction of an image using the standard colors: yellow, cyan, magenta together with black as desired. In copying and proofing the toner particles are applied to a latent electrostatic image.

Other uses are envisioned for the electrostatic liquid developers include: digital color proofing, lithographic printing plates, and resists.

#### EXAMPLES

The following examples wherein the parts and percentages are by weight illustrate but do not limit the invention. In the examples, the melt indices were determined by ASTM D 1238, Procedure A, the average particle sizes by area were determined by a Horiba CAPA-500 centrifugal particle analyzer as described above unless otherwise indicated, conductivities were measured in picomhos (pmho)/cm at five hertz and low voltage, 5.0 volts, and the densities were measured using a Macbeth densitometer model RD 918. Resolution is expressed in the Examples in line pairs/mm (lp/mm). The monofunctional amine additives used in the Examples have the following designations and were all purchased from Aldrich Chemical Co., Milwaukee, Wis.:

TA=tributylamine  
HA=hexylamine  
LA=laurylamine  
DA=dibutylamine

#### CONTROL 1

The following ingredients were placed in a Union Process 01 Attritor, Union Process Company, Akron, Ohio:

| INGREDIENT                                                                                                             | AMOUNT (g) |
|------------------------------------------------------------------------------------------------------------------------|------------|
| Copolymer of ethylene (89%) and methacrylic acid (11%) (PE/MAA):<br>melt index at 190° C. is 100,<br>Acid number is 66 | 200        |
| Sterling NS carbon black,<br>Cabot Corp., Boston, MA                                                                   | 15         |
| Isopar ® -L, nonpolar liquid having<br>a Kauri-butanol value of 27,<br>Exxon Corporation                               | 1000       |

The ingredients were heated to 100° C. +/- 10° C. in the attritor and milled with 0.1875 inch (4.76 mm) diameter steel balls for two hours. The attritor was cooled to room temperature while the milling was continued and then an additional 700 grams of Isopar ®-L were added. Milling was continued for 3 hours to obtain toner particles with an average size of 1.14  $\mu\text{m}$  by area. The particulate media were removed and the dispersion of toner particles was then diluted to 2.0% solids with additional Isopar ®-L. To 2000 grams of the dispersion were added 7.4 grams of a 10% solution of lecithin (Fischer Scientific) in Isopar ®-L. Image quality was determined using a Savin 870copier at standard mode: charging corona set at 6.8 kV and transfer corona set at 8.0 kV using carrier sheets such as Plainwell offset enamel paper, number 3 gloss 60 lb test, Plainwell Paper Co., Plainwell, Mich. Image quality was found to be poor with squash. The results are shown in Table 1 below.

#### CONTROL 2

Toner was prepared as described in Control 1 with the following exceptions: 22 grams of Dalamar ® Yellow YT-858D were used in place of the Sterling NS pigment. The toner was cold ground for 3 hours resulting in average particle size of 1.13  $\mu\text{m}$ . The particulate media was removed and the dispersion of toner particles was then diluted to 1.0% solids with addition of Isopar ®-L. To 1657 grams of the dispersion were added 21 grams of 2.5% lecithin in Isopar ®-L. Image quality was found to be very poor with low resolution, and squash. The results are shown in Table 1 below.

#### CONTROL 3

The following ingredients were placed in a Union Process 01 Attritor Union Process Company, Akron, Ohio:

| INGREDIENT                                                                                                                               | AMOUNT (g) |
|------------------------------------------------------------------------------------------------------------------------------------------|------------|
| Copolymer of ethylene (95%) and acrylic acid (5%), softening point 180° C. (PE/AA), sold as AC540 by Allied Chemical Co., Morristown, NJ | 35.0       |
| Heucophthal Blue G XBT-583D                                                                                                              | 2.63       |
| Heubach, Inc., Newark, NJ                                                                                                                |            |
| Isopar ® -L, nonpolar liquid having a Kauri-butanol value of 27,<br>Exxon Corporation                                                    | 125.0      |

The ingredients were heated to 90° C. to 110° C. and milled with 0.1875 inch (4.76 mm) diameter steel balls for 2 hours. The attritor was cooled to 42° C. to 50° C. While milling was continued and then 88 grams of Isopar ®-H were added. Milling was continued for 21.8 hours to obtain toner particles with an average size of 0.7  $\mu\text{m}$  by area. The particulate media were removed

and the dispersion of toner particles was then diluted to 1% solids with additional Isopar®-L. To 2000 grams of the dispersion were added 4.3 grams of 10% solution of lecithin (Fischer Scientific) in Isopar®-L (90 mg lecithin/g of toner solids). The toner was evaluated as described in Control 1. Image quality was found to be poor with low resolution. Results are shown in Table 1 below.

#### CONTROL 4

Toner was prepared as described in Control 1 with the following exceptions: 200 grams of linear polyethylene having a melt index of 165 (PE) was used instead of the ethylene/methacrylic acid copolymer. 15 grams of Heucophthal Blue G XBT-583D (Heubach Inc., Newark, N.J.) was used in place of the Sterling NS pigment and 2255 grams of Isopar®-L were added. The toner was heated for 20 hours and cold ground for 2 hours resulting in average particle size of 1.63  $\mu\text{m}$  by area. The toner was charged with 10.0 grams of 10% lecithin in Isopar®-L. Image quality was found to be very poor with very poor resolution. Results are shown in Table 1 below.

#### CONTROL 5

Toner was prepared as described in Control 3 with the following exceptions: 35 grams of polystyrene (PS) (Polysciences, Inc., Polystyrene Ultrafine Powder CAT #15790, Warrington, Pa.) was used instead of the ethylene/acrylic acid copolymer. The toner was cold ground for 166 hours resulting in average particle size of 3.8  $\mu\text{m}$  as measured by the Malvern 3600E particle sizer. The toner was charged with 9.23 grams of (10%) lecithin (52 mg/g). Image quality was found to be very poor with low resolution, uneven toning, uneven solids, severe flow and beading, and high squash. Results are shown in Table 1 below.

#### EXAMPLE 1

Toner was prepared as described in Control 1 except that to 2000 g of the dispersion 7.14 g of 10% lecithin in Isopar®-L and 28 grams of 0.1 M TA in Isopar®-L were added image quality was substantially improved compared to Control 1 with reduced squash. Results are shown in Table 1 below.

#### EXAMPLE 2

Toner was prepared as described in Control 1 except that to 2000 g of the dispersion 7.14 g of 10% lecithin in Isopar®-L and 28 grams of 0.1 M HA in Isopar®-L were added. Image quality was substantially improved compared to Control 1 with reduced squash. Results are shown in Table 1 below.

#### EXAMPLE 3

Toner was prepared as described in Control 1 except that to 2000 g of the dispersion 7.14 g of 10% lecithin in Isopar®-L and 28 grams of 0.1 M LA in Isopar®-L were added. Image quality was substantially improved compared to Control 1 with reduced squash. Results are shown in Table 1 below.

#### EXAMPLE 4

Toner was prepared as described in Control 2 except that to 1657 g of the dispersion 21 g of 2.5% lecithin in Isopar®-L and 21 grams of 0.1 M HA in Isopar®-L were added. Image quality was substantially improved

compared to Control 2 with reduced squash. Results are shown in Table 1 below.

#### EXAMPLE 5

Toner was prepared as described in Control 3 except that to 2000 g of the dispersion 4.3 g of 10% lecithin in Isopar®-L and 0.5 gram of HA were added. Image quality was substantially improved compared to Control 3 with improved resolution, density, and evenness of copy and reduced flow, and beading. Results are shown in Table 1 below.

#### EXAMPLE 6

Toner was prepared as described in Control 4 except that to 2000 g of the dispersion 10 g of 10% lecithin in Isopar®-L and 0.5 gram of HA were added. Image quality was substantially improved compared to Control 4. Results are shown in Table 1 below.

#### EXAMPLE 7

Toner was prepared as described in Control 5 except that to 2000 g of the dispersion 9.23 g of 10% lecithin in Isopar®-L and 20.4 grams (120 mg/g) of a 10% solution of HA in Isopar®-L were added image quality was substantially improved compared to Control 5 with improved resolution evenness of copy, reduced flow and beading, reduced squash, and improved density. Results are shown in Table 1 below.

#### CONTROL 6

The following ingredients were placed in a Union Process 01 Attritor Union Process Company, Akron, Ohio:

| INGREDIENT                                                                       | AMOUNT (g) |
|----------------------------------------------------------------------------------|------------|
| Copolymer of ethylene (89%) and methacrylic acid (11%) described in Control 1    | 35         |
| Isopar®-L, nonpolar liquid having a Kauri-butanol value of 27, Exxon Corporation | 125        |

The ingredients were heated to 90° C. to 110° C. and milled with 0.1875 inch (4.76 mm) diameter steel balls for 1 hour. The attritor was cooled to 42° C. to 50° C. While milling was continued and then 88 grams of Isopar®-H (Exxon Corp.) were added. Milling was continued for 5 hours to obtain toner particles with an average size of 17  $\mu\text{m}$  as determined on the Malvern 3600 E particle Sizer. The particulate media were removed and the dispersion of toner particles was then diluted to 2% solids with additional Isopar®-L and a charge director compound such as 80 grams of 10% solution of Emphos®D7O-30C. sodium salt of a phosphoglyceride, Witco Chemical Corp., New York, N.Y. in Isopar®-L was added to 2000 grams of the developer. The toner was evaluated as described in Control 1. Image density was found to be poor. Results are shown in Table 1 below.

#### EXAMPLE 8

Toner was prepared as described in Control 6 except that 28 grams of 0.1 M DA in Isopar®-L were added after the charge director compound. Image density was improved compared to Control 6. Results are shown in Table 1 below.

TABLE 1

| Ex. or Con-trol | Resin  | Pig-ment Type | Amine Adjuvant | Cond. Bulk | Resol-ution (lp/mm) | Trans-fer Eff. % |
|-----------------|--------|---------------|----------------|------------|---------------------|------------------|
| C1              | PE/MAA | Black         | None           | 40         | 8                   | 89               |
| C2              | PE/MAA | Yellow        | None           | 39         | 4                   | 58               |
| C3              | PE/AA  | Cyan          | None           | 30         | 3                   | 41               |
| C4              | PE     | Cyan          | None           | 49         | 3                   | 30               |
| C5              | PS     | Cyan          | None           | 50         | 2-4                 | 47               |
| C6              | PE/MAA | None          | None           | —          | 4                   | 100              |
| E1              | PE/MAA | Black         | TA             | 46         | 9                   | 89               |
| E2              | PE/MAA | Black         | HA             | 39         | 9                   | 74               |
| E3              | PE/MAA | Black         | LA             | 46         | 10                  | 88               |
| E4              | PE/MAA | Yellow        | HA             | 37         | 5.6                 | 64               |
| E5              | PE/AA  | Cyan          | HA             | 34         | 5                   | 90               |
| E6              | PE     | Cyan          | HA             | 54         | 4                   | 90               |
| E7              | PS     | Cyan          | HA             | 75         | 5-7                 | 62               |
| E8              | PE/MAA | None          | DA             | —          | 4                   | 100              |

We claim:

1. A negative electrostatic liquid developer consisting essentially of:
  - (A) a nonpolar liquid having a Kauri-butanol value of less than 30, present in a major amount,
  - (B) thermoplastic resin particles having an average by area particle size of less than 10  $\mu\text{m}$ ,
  - (C) a charge director compound, and
  - (D) at least one organic monofunctional amine compound of the formula:  $\text{R}_n\text{NH}_{3-n}$  wherein R is alkyl, cycloalkyl, or alkylene, said alkyl, cycloalkyl, or alkylene group being of 1 to 50 carbon atoms, and n is an integer of 1 to 3, the sole active substituent present is the amine group.
2. An electrostatic liquid developer according to claim 1 wherein the monofunctional amine compound is of the formula  $\text{R}_n\text{NH}_{3-n}$  and R is an alkyl group of 1 to 50 carbon atoms, and n is an integer of 1 to 3.
3. An electrostatic liquid developer according to claim 2 wherein the monofunctional amine is tributylamine.
4. An electrostatic liquid developer according to claim 2 wherein the monofunctional amine is hexylamine.
5. An electrostatic liquid developer according to claim 2 wherein the monofunctional amine is laurylamine.
6. An electrostatic liquid developer according to claim 1 wherein component (A) is present in 99.9 to 85% by weight, component (B) is present in 0.1 to 15% by weight, based on the total weight of the developer, component (C) is present in an amount of 0.1 to 1000 mg/g developer solids, and monofunctional amine component (D) is present in an amount of 0.1 to 1000 mg/g developer solids.
7. An electrostatic liquid developer according to claim 1 containing up to about 60% by weight of a colorant based on the weight of resin.

8. An electrostatic liquid developer according to claim 7 wherein the colorant is a pigment.
9. An electrostatic liquid developer according to claim 8 wherein the percent pigment in the thermoplastic resin is 1% to 60% by weight based on the weight of resin.
10. An electrostatic liquid developer according to claim 7 wherein the colorant is a dye.
11. An electrostatic liquid developer according to claim 1 wherein a fine particle size oxide is present.
12. An electrostatic liquid developer according to claim 1 wherein present in the thermoplastic resin is a metallic soap.
13. A negative electrostatic liquid developer consisting essentially of:
  - (A) a nonpolar liquid having a Kauri-butanol value of less than 30, present in a major amount,
  - (B) thermoplastic resin particles of a copolymer of ethylene and an  $\alpha,\beta$ -ethylenically unsaturated acid selected from the group consisting of acrylic acid and methacrylic acid having an average by area particle size of less than 10  $\mu\text{m}$ ,
  - (C) a charge director compound, and
  - (D) at least one organic monofunctional amine compound of the formula:  $\text{R}_n\text{NH}_{3-n}$  wherein R is alkyl, cycloalkyl, or alkylene, said alkyl, cycloalkyl, or alkylene group being of 1 to 50 carbon atoms, and n is an integer of 1 to 3, the sole active substituent present is the amine group.
14. A negative electrostatic liquid developer consisting essentially of:
  - (A) a nonpolar liquid having a Kauri-butanol value of less than 30, present in a major amount,
  - (B) thermoplastic resin particles of a copolymer of ethylene (80 to 99.9%)/acrylic or methacrylic acid (20 to 0%)/alkyl ester of acrylic or methacrylic acid wherein alkyl is 1 to 5 carbon atoms (0 to 20%) having an average by area particle size of less than 10  $\mu\text{m}$ ,
  - (C) a charge director compound, and
  - (D) at least one organic monofunctional amine compound of the formula:  $\text{R}_n\text{NH}_{3-n}$  wherein R is alkyl, cycloalkyl, or alkylene, said alkyl, cycloalkyl, or alkylene group being of 1 to 50 carbon atoms, and n is an integer of 1 to 3, the sole active substituent present is the amine group.
15. An electrostatic liquid developer according to claim 13 wherein the thermoplastic resin is a copolymer of ethylene (89%)/methacrylic acid (11%) having a melt index at 190° C. of 100.
16. An electrostatic liquid developer according to claim 13 wherein the particles have an average by area particle size of less than 5  $\mu\text{m}$ .
17. An electrostatic liquid developer according to claim 13 wherein component (C) is lecithin.
18. An electrostatic liquid developer according to claim 13 wherein component (C) is the alkali metal salt of a phosphoglyceride.

\* \* \* \* \*

UNITED STATES PATENT AND TRADEMARK OFFICE  
CERTIFICATE OF CORRECTION

PATENT NO. 4,935,328

DATED : June 19, 1990

INVENTOR(S) : Enrico Selva, et al.

It is certified that error appears in the above-identified patent and that said Letters Patent  
is hereby corrected as shown below:

In column 21, line 26, the patent reads "(2 x 10 1)" and should  
read --(2 x 20 1)--.

In column 26, line 43, the patent reads "N<sub>2</sub>SO<sub>4</sub>" and should read  
--Na<sub>2</sub>SO<sub>4</sub>--

Signed and Sealed this  
Ninth Day of February, 1993

Attest:

STEPHEN G. KUNIN

Attesting Officer

Acting Commissioner of Patents and Trademarks